

# United States Patent Office

3,542,745  
Patented Nov. 24, 1970

1

3,542,745

## TERPOLYAMIDES USEFUL IN PREPARING TEXTILE FIBERS CONSISTING ESSENTIALLY OF NYLON 66, NYLON 6, AND NYLON 2-6IA

Rupert J. Snooks, Jr., Gulf Breeze, Fla., assignor to Monsanto Company, St. Louis, Mo., a corporation of Delaware

No Drawing. Filed Oct. 29, 1968, Ser. No. 771,617  
Int. Cl. C08g 20/12, 20/20

U.S. Cl. 260—78

9 Claims

### ABSTRACT OF THE DISCLOSURE

Textile fibers spun and drawn from a synthetic linear polyamide having a polymer chain consisting of at least 93 weight percent



units, from 0.25 to 3 weight percent



units and from 0.5 to 4 weight percent



units in which  $n$  is 2 to 6 are of improved quality and dyeability.

### BACKGROUND OF THE INVENTION

Nylon 66 (polyhexamethylene adipamide) is well known for its superior textile properties. However, it does have certain disadvantages when used in providing textile yarns. One disadvantage is that when nylon 66 is processed into drawn yarn, the yarn tends to contain one or more short segments along its length which have a denier greater than that intended. These segments are flaws in the yarn which result from defects in the polymer or from imperfections in the spinning operation. In knitting operations as the yarn passes through eyes of knitting machines such segments bind in the eyes causing the yarn to break. The term "internal quality" has been coined to reflect the number of these segments which exist along the length of the yarn and is determined by passing a sample of the yarn through a passage defined by two pairs of parallel blades, one pair being positioned parallel above the other pair and at a 90° angle thereto, i.e., #. The spacing between the parallel blades of each pair is set to permit yarn of a selected denier to pass through the passage defined by the blades without obstruction. However, if the yarn contains segments of larger denier, the blades cut the yarn. The number of cuts (breaks) in the yarn which occur in passing the yarn through the passage divided by the number of pounds of yarn involved is expressed as the internal quality (breaks per pound) of the yarn. In providing yarn for use in knitting operations, the internal quality of the yarn is of major concern.

Another disadvantage in processing nylon 66 into textile yarns is that fibers or fabrics prepared therefrom do not dye rapidly or uniformly.

An object of the present invention therefore is to provide a nylon yarn having physical properties comparable to nylon 66 as well as having improved internal quality, a high dye absorption rate and improved uniformity of dyeing.

2

### SUMMARY OF THE INVENTION

The above and other objects are accomplished by providing a textile filament spun and drawn from a synthetic linear terpolyamide having a polymer chain consisting of from about 93 to 99.25 weight percent of the repeating unit



10 from 0.25 to 3 weight percent of the repeating unit



15 and from 0.5 to 4 weight percent of the repeating unit



20

in which  $n$  is 2 to 6, wherein said 66 units, 6 units and  $n\text{IA}$  units are randomly distributed throughout said polymer chain.

25 The terpolyamides may be prepared by polymerizing a mixture consisting of appropriate amounts of the terpolyamide-forming components in the manner well known in the art and commonly employed in the manufacture of nylon 66. Thus, the terpolyamides may be prepared according to a modified nylon 66 process 30 wherein appropriate amounts of  $\epsilon$ -caprolactam and the selected diamine salt of isophthalic acid are added either separately or in combination to the nylon 66 salt at any point in the process prior to polymerization.

35 The amount of  $\epsilon$ -caprolactam or  $\epsilon$ -amino-caproic acid used in forming the terpolyamides preferably ranges from about 0.25 to 3 mole percent, based on the total weight of the terpolyamide-forming components. Although slightly greater amounts could possibly be used 40 without altering the character of the resulting terpolyamide, the improvement, if any, achieved thereby would be outweighed by cost considerations. The amount of diamine-isophthalic acid salt used in preparing the terpolyamides preferably ranges from about 0.5 to 4 mole percent. If greater amounts are employed, the shrinkage 45 and other physical properties of the terpolyamides are noticeably changed.

The invention is further illustrated by the following examples.

### PREFERRED EMBODIMENTS OF THE INVENTION

#### Example 1

55 Dry  $\epsilon$ -caprolactam monomer was added to 40% aqueous solution of hexamethylene diammonium isophthalate (nylon 6IA salt) and this combination was added to normal 50% aqueous solution of nylon 66 salt prior to beginning evaporation. The quantities of caprolactam and nylon 6IA salt were selected to produce a 250-pound 60 batch of terpolyamide containing 4 weight percent 6IA units, 0.5 weight percent 6 units and 95.5 weight percent 66 units. The salt mixture was charged to a stainless steel evaporator and heated to 137° C. while maintaining a pressure within the evaporator of 13 p.s.i.g. to obtain a 75% solution. The solution is then transferred to a stainless steel autoclave wherein the temperature is gradually increased to 270° C. to effect polymerization. When the batch temperature reached 200° C., sufficient 70 30% aqueous  $\text{TiO}_2$  was added to provide 0.3 weight percent in the terpolymer. The molten terpolymer having a melt viscosity of 30 was extruded onto a casting wheel, solidified and cut into chips. The chips were subsequently

charged to a spinning grid, melted at a temperature of 293° C., and pumped at a pressure of 4000 p.s.i.g. through a sand pack filter and 13-hole spinneret to form a bundle of filaments which are quenched by a cross-current flow of air. After cooling, the filament bundle was passed downward over a finish roll for application of finish and wound onto a bobbin. The spun yarn composed of 13 filaments and having a nominal total denier of 123 was drawtwisted using a conventional Whitin RG-4 drawtwister at a draw ratio of 3.51 to 1 to yield 40 denier yarn having  $\frac{1}{2}$  Z twist.

Nylon 66 yarns were also prepared for purposes of comparison according to the procedure just described with the exception that the caprolactam and nylon 6IA salt were omitted. Properties of the yarns were determined and are given in Table I. The internal quality of the yarns was determined by the procedure described above.

TABLE I

|              | Draw ratio | Denier | Elongation | Breaking strength | Tension | Drawtwist performance, breaks and wraps/lb. | Internal quality, bks./lb. |
|--------------|------------|--------|------------|-------------------|---------|---------------------------------------------|----------------------------|
| Nylon 66     | 3.23       | 39.7   | 31.5       | 188               | 4.74    | 0.107                                       | 1.654                      |
| Terpolyamide | 3.51       | 40.1   | 29.3       | 191               | 4.76    | 0.075                                       | 0.417                      |

The results in Table I show that the drawtwist performance and internal quality of the terpolyamide yarns, when compared to nylon 66 yarns, are significantly superior.

In the following examples the dye rate and dye penetration of the yarns were also determined.

The dye rate of the yarns was measured by immersing a skein of yarn weighing 6 grams into a dye bath containing 0.2 gram Orlon Bordeaux RR (Acid Red 296) and 750 ml. of pure water. The dyebath was maintained at a temperature of 89°  $\pm$  1° C. Acid Red 296 is a chromium complex derived from



and is substantially equivalent to Pernon Fast Red 3BS which is no longer produced. A Beckman DK2A recording spectrophotometer measures and records the concentration of dye in the bath as a function of time. From these data the time required for the yarn sample to reach half of its saturation value was calculated.

The dye penetration of the yarns was measured by immersing a skein of yarn weighing 5 grams into a dye-bath containing 0.025 gram of Color Index Number Acid Blue 113 (Pontacyl Fast Blue 5R) and 1000 ml. of pure water. The dyebath was maintained at a temperature between 80°-90° C. Pontacyl Fast Blue 5R has the structure



After 30 minutes the yarn sample was dried, cross-sectioned and the percent radial penetration measured microscopically.

According to an alternative procedure for measuring the dye penetration and dye rate of yarns a skein of yarn, after scouring to remove the spin finish, was dyed in Chromacyl Black w solution containing 0.25 weight percent dye, 0.5 weight percent ammonia and 40 ml. of pure water per gram of yarn. When the yarn sample was immersed in the dyebath, the dyebath temperature was 70° F. The bath was increased to 190° F. in 10 minutes and then to 212° F. in 10 additional minutes. Dyeing was continued for 60 minutes at 212° F. The yarn sample was then rinsed, dried and the reflectance thereof measured using a reflectometer as follows: the yarn sample was

placed in a rotating cell and light is impinged on the yarn and the reflected light was measured and a value determined. The lower the value, the greater the dye depth and the diffusivity of the fiber. The standard deviation of the samples were determined statistically using 26 randomly selected bobbins from the polymer prepared. Chromacyl Black w (Acid Black 52) is formed by complexing two atoms of chromium with three moles of:



It will be observed from the data obtained in Examples 2 and 3 that the Chromacyl Black dye value determined

for each composition correlates closely with the percent diameter penetration value and the time to half dye value determined therefor. Thus, for example, a composition having a lesser time to half dye value and a greater percent diameter penetration value, will also have a lesser Chromacyl Black dye depth value. However, the determination of the time to half dye values and the percent diameter penetration values are tedious analytical procedures, whereas the determination of Chromacyl Black dye depth values is a relatively simple procedure.

#### Example 2

A series of yarns, each having a different composition, were prepared according to the procedure of Example 1, with the exception that a 26-hole spinneret was employed rather than a 13-hole spinneret and the yarn was drawn to a denier of 30. The composition of each yarn in the series is given in Table II. The dye penetration, dye rate and Black Chromacyl dye depth values of each yarn were determined following the procedures described above and the drawtwist performance of each yarn was observed. The results are given in Table II.

TABLE II

| Yarn composition, weight percent | Drawtwist performance, breaks/lb. | Colormaster Black dye depth and standard deviation | Percent diameter penetration with Acid Blue 113 | Time to half dye, min. |
|----------------------------------|-----------------------------------|----------------------------------------------------|-------------------------------------------------|------------------------|
| 66 6IA 6                         |                                   |                                                    |                                                 |                        |
| 100-----                         | 0.064                             | 204-29.1                                           | 54.9                                            | 3.65                   |
| 96.5-----3.5                     | 0.046                             | 248-37.9                                           | 55.4                                            | 2.9                    |
| 95-----3.5 1.5                   | 0.028                             | 118-30.1                                           | 72.3                                            | 1.5                    |
| 94-----6 -----                   | 0.084                             | 227-33.7                                           | 53.3                                            | -----                  |

These results show that yarn prepared from the terpolyamides of the present invention have superior drawtwist performance, dye rate and dye penetration, when compared to yarns prepared from nylon 66 or copolymers containing 66 and 6IA units in which the 6IA units comprise 6 weight percent of 3.5 weight percent of said copolymer.

#### Example 3

A series of yarns, each having a different composition, were prepared according to the procedure of Example 1 and tested in the same manner as described in Example 2. The results of these tests are given in Table III.

TABLE III

| Yarn composition, weight percent |     |     |     | Drawtwist performance, breaks/lb. | Internal quality, breaks/lb. | Draw ratio | Colormaster dye depth, Chromacyl black | Diameter penetration, percent | Time to half dye, seconds |
|----------------------------------|-----|-----|-----|-----------------------------------|------------------------------|------------|----------------------------------------|-------------------------------|---------------------------|
| 66                               | 6IA | 6   | 4IA | 2IA                               |                              |            |                                        |                               |                           |
| 97                               | 3.0 |     |     |                                   | 0.16                         | 8.00       | 3.22                                   | 365                           | 33 287                    |
| 95                               | 3.0 | 2.0 |     |                                   | 0.04                         | 0.46       | 3.22                                   | 295                           | 55.3 287                  |
| 95                               | 2.0 | 3.0 |     |                                   | 0.06                         | 0.66       | 3.99                                   | 237                           | 71.0 187                  |
| 94                               | 6.0 |     |     |                                   | 0.06                         | 0.92       | 3.22                                   | 300                           | 46.7 262                  |
| 96                               | 4.0 |     |     |                                   | 0.06                         | (1)        | 3.22                                   | 349                           |                           |
| 94                               | 4.0 | 2.0 |     |                                   | 0.04                         | 0.57       | 3.22                                   | 263                           | 68.1 200                  |
| 94                               | 2.0 | 4.0 |     |                                   | 0.04                         | 0.82       | 3.99                                   | 224                           | 70.6 188                  |
| 95                               |     | 1.5 | 3.5 |                                   | 0.05                         | 0.88       | 3.99                                   | 144                           | 2 ~100 2 ~125-150         |

<sup>1</sup> Unrunnable.<sup>2</sup> Estimated.

The results in Table III further demonstrate that yarn prepared from the terpolyamides of the present invention have excellent drawtwist performance, internal quality and dye characteristics. Surprisingly, yarns composed of 66-6-4IA and 66-6-2IA dyed darker with the Chromacyl Black dye than the yarns composed of 66, 66-61A or 66-6-6IA even though the draw ratio of the yarns was considerably higher. Moreover, an increase in spinning production is realized in spinning yarns composed of 66-6-4IA and 66-6-2IA since at constant spinning speeds the draw ratio required to produce a given yarn elongation (denier) is higher than that required for the other yarns.

What is claimed is:

1. A linear synthetic terpolyamide having a polymer chain consisting essentially of 93 to 99.25 weight percent or randomly repeating units of the structure



0.25 to 3 weight percent of randomly repeating units of the structure



and 0.50 to 4 weight percent of randomly repeating units of the structure



in which  $n$  is an integer from 2 to 6.

2. The terpolyamide of claim 1, wherein  $n$  is 6.
3. The terpolyamide of claim 1, wherein  $n$  is 4.
4. The terpolyamide of claim 1, wherein  $n$  is 2.
5. A nylon filament consisting essentially of the terpolyamide of claim 1.
6. The nylon filament of claim 5, wherein the terpolyamide consists essentially of 94 weight percent



units in which  $n$  is an integer from 2 to 6.

7. The nylon filament of claim 6, wherein  $n$  is 6.
8. The nylon filament of claim 7, wherein  $n$  is 4.
9. The nylon filament of claim 7, wherein  $n$  is 2.

#### References Cited

##### UNITED STATES PATENTS

|           |        |               |         |
|-----------|--------|---------------|---------|
| 2,071,253 | 2/1937 | Carothers     | 260-78  |
| 2,252,555 | 8/1941 | Carothers     | 260-78  |
| 2,252,557 | 8/1941 | Czerwin       | 260-78  |
| 3,310,534 | 3/1967 | Brignac       | 260-78  |
| 3,322,731 | 5/1967 | Cook et al.   | 260-78  |
| 3,383,369 | 5/1968 | Ridgway       | 260-78  |
| 3,399,108 | 8/1968 | Olson         | 161-173 |
| 3,454,536 | 7/1969 | Schade et al. | 260-78  |

##### FOREIGN PATENTS

|           |        |                |
|-----------|--------|----------------|
| 1,025,098 | 4/1966 | Great Britain. |
| 1,114,541 | 5/1968 | Great Britain. |

50 WILLIAM H. SHORT, Primary Examiner

H. SCHAIN, Assistant Examiner

U.S. Cl. X.R.

55 8-55; 57-140